

## UNITED STATES PATENT OFFICE

2,044,721

## MANUFACTURE OF LUBRICATING OIL

Francis X. Govers, Vincennes, Ind., assignor to  
Indian Refining Company, Lawrenceville, Ill.,  
a corporation of Maine

No Drawing. Application March 29, 1933,  
Serial No. 663,341

3 Claims. (Cl. 196—17)

This invention relates to the manufacture of mineral lubricating oils and more particularly to the manufacture of high viscosity index, low pour test lubricating oil from wax bearing mineral oils.

In its broadest aspect, the invention contemplates an improved process of treating hydrocarbon oils, particularly paraffin-bearing lubricating fractions of petroleum with solvents to selectively produce therefrom low pour test lubricating oils characterized by having a desired viscosity temperature relationship and improved lubricating qualities. The invention contemplates a process of manufacturing lubricating oils having low pour and cloud tests, low sulphur content, low Conradson carbon content, relatively high viscosity index and freedom from bodies of little or no lubricating value.

Lubricating oils, as ordinarily made from naphthalene-base crudes, have low pour and cloud tests, low Conradson carbon content, but have low viscosity indices and fairly high sulphur content. On the other hand, lubricating oils, as ordinarily made from paraffin-base crudes of the Pennsylvania type, have high pour and cloud tests, high Conradson carbon content and fairly high sulphur content, depending on the source of particular crude used. Oils derived from mixed base crudes fall somewhere between these limits although usually high in sulphur content. Oils of the Pennsylvania type, as well as those derived from mixed base crude sources, are difficult to refine without undue loss and impairment of their lubricative value. In all cases, it is difficult, by methods now employed, to reduce the sulphur content of these lubricating oil fractions to a desired point, regardless of their source of crude.

I have discovered that by the use of the methods herein disclosed lubricating oils of any desired viscosity index and scale of purification coupled with low pour test and low cloud test, can be made from mixed-base or paraffin-base crudes and the oils so produced are characterized further by low Conradson carbon and low sulphur content. The obtaining of oils having these desired qualities does not depend on methods involving redistillation or acid treatment, although such redistillation or acid treatment can be coupled with the methods herein disclosed if so desired.

Lubricating oils of high viscosity index are characterized by having a relatively narrow increase in viscosity with respect to temperature. Such oils have the property of possessing the desired viscosity at elevated temperature with not too great a loss of mobility at very low tempera-

ture. The viscosity index of a given oil is readily determined by resorting to the method of Dean and Davis, published on pages 618-619 of the 1929 issue of Chemical and Metallurgical Engineering.

More specifically the invention comprises mixing with a wax-bearing fraction of a mineral oil a solvent mixture composed of aniline and a modifying solvent selected from the group comprising isopropyl ether, ethyl ether, benzol, toluol, and the like, in such proportion to each other and to the oil that the mixture has substantially complete solvent action on the oil at temperatures of around 100° F., and at temperatures of around 0° F. substantially complete solvent action on the liquid hydrocarbons therein but substantially no solvent action on the solid hydrocarbons therein and of such a nature that upon cooling a solution of the mineral oil fraction in such solvent mixture to 0° F. and removing the solid hydrocarbons so precipitated and the solvent liquid the resulting oil has a cold test of substantially 0° F. or below.

The mixture is then chilled to form a precipitate of solid or semi-solid material comprising suspended wax or solid hydrocarbons which are insoluble in, and immiscible with, the desired solvent mixture. The mother liquor is separated from the chilled mixture, advantageously by filtration. The separated mass of solid hydrocarbons is then washed free of mother liquor containing dissolved oil by additional quantities of chilled solvent liquid of approximately the same composition as used in the original mix.

A portion of the first part of this wash filtrate may be added to the original filtrate. The extent of such addition depending on the amount or percentage of oil contained in such wash filtrate.

From the original filtrate or mixture of original filtrate and wash filtrate is then evaporated one of the component solvents in an amount sufficient to effect the desired alteration in the selective solvent action of the mixture. If desired this resulting mixture may be treated with additional amounts of the remaining solvent component.

This resulting mixture of altered composition may be cooled or chilled to still further affect its solvent action and is allowed to stand and effect a sharp separation into two layers. The upper layer contains oils characterized by relatively high viscosity index and the lower layer contains oils of relatively low viscosity index.

The amount and character of the separation is influenced by the amount of alteration in the

- percentage composition of the component parts comprising the solvent mix and the temperature to which such altered composition mixture is chilled. If desired the modifying solvent may be removed in successive stages, subjecting the remaining mixture of dissolved oil and solvent to cooling in each instance to thereby successively separate fractions of differing characteristics as may be desired.
- 10 It is contemplated that the wax-bearing fraction may be subjected to preliminary refining either with acid or by extraction with a suitable solvent such as the selective solvent component of the mixture used in the subsequent steps. The 15 resulting treated fraction is then dewaxed by means of a chilled selective solvent mixture composed of the selective solvent and a modifying solvent, followed by the separation of the dewaxed fraction into oils of differing viscosity indices by 20 means of evaporation in whole or part of the modifying solvent. The solvent component of relatively high selectivity may be aniline, or a solvent of like solvent nature and the modifying solvent of relatively less selectivity may be iso- 25 propyl ether, ethyl ether, toluol, benzol, or a solvent of like solvent nature.

As an example of the process:

- An acid treated wax distillate having the following approximate characteristics, gravity 26° 30 Bé., viscosity of 70 Saybolt universal seconds at 210° F., and a pour test of 95° F. is well mixed with isopropyl ether. Following this, aniline is then added. The proportions of these two solvents used comprises about 60 parts of ether to 35 about 40 parts of aniline. The mixture is well stirred, chilled to -20° F., and while maintained in this chilled condition, introduced to a pressure type filter such as described in my copending application, Serial No. 585,844, wherein the solid 40 hydrocarbons are separated to produce a filtrate substantially free from dissolved wax and solid hydrocarbons.

- The filter cake, without removal from the filter, is washed with additional solvent liquid mixture of substantially the same composition and which has been chilled to a temperature of -20° F. This wash filtrate is used for part of the solvent mixture in a succeeding batch, allowance being made for the oil contained therein.

- 50 The wax slurry is drawn off from the filter and the solvent removed by evaporation or distillation in a reducing or non-oxidizing atmosphere, such as carbon dioxide for example. The wax, free from solvent, is then steam treated in the 55 presence of clay and contact filtered. The resulting wax is practically water white and will have a melting point of approximately 138° F.

- From the dewaxed filtrate a portion, or substantially all, of the isopropyl ether is evaporated, depending upon the degree of separation desired. The resulting mixture may be chilled to any temperature desired, upon which separation into two layers will occur. One layer will comprise the high viscosity index constituents, while the other 65 layer will contain the low viscosity index constituents.

- In the event that substantially all of the isopropyl ether is evaporated from the dewaxed filtrate, it may be advantageous to extract the resulting mixture with an additional quantity of aniline. This extraction may be carried out by countercurrent methods at a temperature of around 60° F., for example, using about one part of aniline to two parts of oil. As a result of this 70 extraction, the oil will, upon settling, be separated

into two layers, one of which contains relatively high viscosity oil while the other contains relatively low viscosity oil.

The aniline is advantageously removed from the separated layers by steam distillation and recovered for further use. The remaining oil may then be finished up by contact filtration in the usual manner.

The high viscosity index fraction obtained in the above manner will have a gravity of about 10 30.4 Bé., a viscosity of about 65 Saybolt universal seconds at 210° F., a viscosity index of not less than 100, a pour test of not higher than -15° F., a Conradson carbon content not greater than 0.02% and a sulphur content not greater 15 than 0.09%.

The invention is not limited to the production of final products of the characteristics of those produced in the examples given above. Products of varying characteristics may be produced by 20 varying the proportions of solvent liquids and their concentration and the temperature at which the treating steps are carried out.

Furthermore, the invention is not limited to the treatment of wax distillate such as given in 25 the examples herein but is adapted to the treatment of other paraffin-containing fractions, precipitates or materials somewhat similar in nature derived in various ways from mineral oils.

Thus my invention is applicable to the treat- 30 ment of hydrogenation products resulting from the hydrogenation of carbonaceous materials, or mineral oils including liquid or solid hydrocarbon fractions derived from mineral oils. Hydro- 35 genation products may contain substantial quantities of waxy or paraffin material as well as other constituents of relatively low lubricating value. By treating such products in accordance with my invention, final products of desired characteristics can be obtained. 40

The invention is not restricted to any particular operating condition such as that of temperature, or the composition of the solvent mixtures employed since these conditions may advantageously be varied, depending upon the nature of the frac- 45 tion undergoing treatment as well as upon the particular characteristics desired in the final product.

It is also contemplated, in many instances, that it may be of advantage to carry on the filtration 50 step in the presence of a comminuted solid filter-aid material. Such material may be admixed with the chilled mixture of oil and solvent liquid prior to introduction to the filtering means.

Obviously many modifications and variations 55 of the invention, as hereinbefore set forth, may be made without departing from the spirit and scope thereof, and therefore only such limitations should be imposed as are indicated in the ap- 60 pended claims.

I claim:

1. The process of manufacturing viscous lubricating oil having a pour test of 0° F. and below and a viscosity index of 100 and above from viscous wax-bearing mineral oil comprising mixing 65 with the oil a solvent consisting of about 40% aniline and 60% isopropyl ether in proportion with the oil such that at 0° F. and below the mixture has substantially complete solvent ac- 70 tion on the liquid hydrocarbons and substantially no solvent action on the solid hydrocarbons, and such that upon cooling the mixture of solvent and oil to 0° F. and removing the solid hydrocarbons precipitated and the solvent liquid, the resulting oil has a cold test of around 0° F., chilling 75

the mixture to a temperature of 0° F. and below to precipitate the wax, removing the precipitated wax, vaporizing a large portion of the isopropyl ether from the dewaxed mixture, extracting the 5 remaining mixture with aniline, a portion of which comprises aniline used in the dewaxing step, separating the mixture while at a temperature of around 60° F. into extract and raffinate phases, removing the raffinate phase, and removing 10 the solvent from said raffinate phase to produce oil having the aforesaid characteristics.

2. The process of dewaxing viscous wax-bearing oil to produce oil having a pour test of 0° F. and below which comprises mixing the oil with 15 a solvent consisting of about 40% aniline and 60% isopropyl ether in proportion with the oil such that at 0° F. and below the mixture has substantially complete solvent action on the liquid hydrocarbons and substantially no solvent 20 action on the solid hydrocarbons, and such that upon cooling the mixture of solvent and oil to 0° F. and removing the solid hydrocarbons precipitated and the solvent liquid, the resulting oil has a cold test of around 0° F., chilling the 25 mixture to a temperature of 0° F. and below to

precipitate the wax, and removing the precipitated wax therefrom.

3. The process of manufacturing high viscosity index lubricating oil having a low pour test from wax-bearing mineral oil which comprises mixing with the oil a solvent liquid mixture composed of aniline and a modifying solvent, such as isopropyl ether, having substantially no selective action as between constituents of the oil of differing viscosity indices and mixed with each other and with the oil in proportions such that at temperatures of around 0° F. the mixture has substantially complete solvent action on the oil, and substantially no solvent action on the wax, chilling the mixture to precipitate wax constituents of the oil, removing the wax thus precipitated, removing from the resulting dewaxed mixture a suitable portion of the modifying solvent to thereby render the remaining solvent liquid selective as between constituents of the oil of 20 differing viscosity indices, and separating from the remaining mixture a fraction of desired viscosity index and low pour test.

FRANCIS X. GOVERS. 25